# EUROPEAN PATENT SPECIFICATION

(11) **EP 1 584 696 B1**
(45) Date of publication and mention of the grant of the patent: **08.11.2006**
(21) Application number: 02762779.3
(22) Date of filing: 15.08.2002
(51) Int. Cl.: C22C 1/10, B22F 1/00, C22C 5/06, H01H 1/02, C22C 32/00

(54) **METHOD FOR PRODUCING Ag-OXIDE-BASED ELECTRIC CONTACT MATERIAL AND ITS PRODUCT**
HERSTELLUNGSVERFAHREN FÜR ELEKTRISCHES KONTAKTMATERIAL AUF Ag-OXIDBASIS UND DESSEN PRODUKT
PROCEDE DE PRODUCTION D'UN MATERIAU DE CONTACT ELECTRIQUE A BASE D'OXYDE-AG ET SON PRODUIT

(43) Date of publication of application: 12.10.2005
(73) Proprietor: Tokuriki Honten Company Limited, Chiyoda-ku Tokyo 101-0044 (JP); Fuji Electric FA Components & Systems Co., Ltd., Tokyo 141-0032 (JP)
(72) Inventor: SATO, Sadao, c/o Tokuriki Honten Co., Ltd., Tokyo 101-0044 (JP); KUMITA, Hideo, c/o Tokuriki Honten Co., Ltd., Tokyo 101-0044 (JP); TSUDA, Kohei, c/o Tokuriki Honten Co., Ltd., Tokyo 101-0044 (JP); YAMASHITA, Mitsuo, c/o Fuji Electric Co., Ltd., Kawasaki-shi, Kanagawa 210-0856 (JP); SHIOKAWA, Kunio, c/o Fuji Electric Co., Ltd., Kawasaki-shi, Kanagawa 210-0856 (JP); KAMIURA, Kenichi, c/o Fuji Electric Co., Ltd., Kawasaki-shi, Kanagawa 210-0856 (JP); SEKIGUCHI, Kiyoshi, c/o Fuji Electric Co., Ltd., Kawasaki-shi, Kanagawa 210-0856 (JP)
(74) Representative: Koch, Günther
(86) International application number: PCT/JP2002/008294
(87) International publication number: WO 2004/016818

(56) References cited:
- EP-A- 0 508 055
- EP-A- 0 877 403
- JP-A- 9 089 727
- JP-A- 54 002 234
- JP-A- 58 100 650
- JP-A- 59 219 432
- JP-A- 62 241 207
- US-A- 3 874 941

## Description

### Technical Field

This invention relates to an Ag-oxide-based electric contact material having excellent contact reliability, deposition resistance and arc resistance, used for various switches, contactors, breakers and the like, and a method for manufacturing the same.

### Background Art

Among various electric contact materials that have been used, particularly Ag-CdO-based materials have excellent electric properties such as deposition resistance, arc resistance and low contact resistance and therefore there has been a large demand for Ag-CdO-based materials in various fields. These materials have been improved over a long time and many academic researches on these materials have been conducted. These materials and manufacturing techniques have reached, so to speak, the maximum.

Recently, however, the cadmium (Cd) discharge standard provision in Japan, EC Directive on Waste from Electrical and Electronic Equipment (WEEE) and the like have been directed toward disuse of Cd, as already known.

Under such conditions, a Cd-free contact material having excellent electric properties that can replace Ag-CdO-based electric contact materials have been increasingly demanded.

A contact material free of Ca is disclosed in US-A-3,874,941. In accordance therewith indium oxides are precipitated in the silver matrix as compound oxides with Sn with the progress of the internal oxidation, by adding Sn in more than 0.5 weight percent, thus producing the hard contact material dispersed with refractory oxides. One of the samples comprises Ag-In 10%, Sn 3%, Ni 0.2% which provided an excellent anti-weld characteristic. The method was carried out using an oxygen atmosphere in the furnace during the pressurized internal oxidation step with a pressure of 3atm of oxygen at about 700°C.

Another contact materials free of Ca are disclosed in EP-A-0 877 403. In accordance with the invention of this patent each contact is formed of a material prepared by inner oxidation of an alloy having the composition of 0.2 to 5.0 wt% of tin, 5.0 to 8,0 wt% of indium, at most 0.5 wt% of iron family metal and remaining part of silver. According to the present invention, 2.0 to 5.0 wt% of tin, which improves welding resistance and 5.0 to 8.0 wt% of indium, which improves ablation resistance, are mixed, whereby welding resistance and ablation resistance of the contact material itself can further be improved. One of the samples contains Sn: 3.2 wt%, In: 6.3 wt%, Ni: 0.2 wt% and remaining part of Ag.

As internal oxidation processing is performed to an alloy formed by adding Sn, In, Sb, Bi or the like to Ag, an internal structure having an oxide precipitated and dispersed therein is provided. However, as a result of research on contact manufacturing conditions, internal oxidation conditions, and damage and exhaustion after contact property evaluation test, it is found that an Ag-rich layer formed on the surface at the time of preparing a contact and an oxide-flocculated layer that is immediately below the Ag-rich layer cause adverse effects such as deposition and increase in temperature of the contact at the time of opening/closing of the contact.

Thus, it is an object of the present invention to solve the problem of disuse of Cd, provide properties equivalent to those of an Ag-CdO-based electric contact material, restrain generation of an Ag-rich layer and an oxide-flocculated layer that is immediately below the Ag-rich layer, which are proper to internal oxidation processing of a Cd-free contact material such as an Ag-(Sn, In, Sb)-based material, and solve various problems such as unevenness in distribution of concentration of added element oxide particles, coarsening of the particles, and flocculation of the particles.

The above mentioned object is solved by a method as claimed in claim 1. The method of claim 1 also in connection with claim 2 can be adventageously used for the production of different Ca-free contact materials, f.i. for an Ag-oxide-based electric contact material made of Sn at a rate of 1 to 5% by weight, In at 3 to 10% by weight, one or more types of Fe, Ni and Co at 0.05 to 1% by weight, and Ag for the remaining part.

The invention of claim 1 also in connection with claim 3 can be used for the production of electric contact material having the novel alloy as claimed in claims 4, 5 and 6, wherein the structure and homogeneity of the oxidy dispersion in the alloy can be specifically improved.

The following is a summary of the invention as explained by the inventor:

In the present invention, the inventor analyzed various elements causing the temperature, oxygen pressure and added element in the internal oxidation mechanism to change the oxidized structure and also reviewed the manufacturing conditions with a broader scope of analysis. Moreover, the inventor reconsidered the contribution of various elements other than Cd to the contact property of the oxide and analyzed various phenomena with respect to a cleaning effect and arc on the surface of an electric contact, for example, properties of an oxide to be added, particularly the temperature characteristic of its steam pressure and the relation between the state of dispersion in Ag and an arc-suppressing phenomenon in an arc generated at the time of opening/closing. Thus, the inventor could confirm the optimum relation of the dispersion in Ag of an oxide containing an added element and composite oxide having electric properties such as deposition resistance, arc resistance and low contact resistance that are equivalent to those of an Ag-CdO-based electric contact material.

On the basis of such confirmation, the inventor paid attention to an Sn oxide and an Sb oxide, which have a higher steam pressure than CdO within a temperature range of approximately 1500 to 4000°C and are less toxic, and confirmed that these oxides exhibit a contact surface cleaning effect equivalent to or higher than that of a CdO-based material.

Moreover, the inventor also confirmed that dispersion of composite oxides of added elements other than Sn into Ag provides a synergistic effect.

Thus, the present invention is provided on the basis of the above-described confirmation. The present invention is characterized in that an oxide of In having a low steam pressure than CdO within a temperature range of approximately 500 to 4000°C is dispersed in an Sn oxide, thereby making the behavior of a synthetic steam pressure of these oxides in the form of a metal composite oxide more approximate to the behavior of the steam pressure of CdO so that their synergistic effect provides excellent contact properties. The present invention is also characterized in that as a measure for restraining generation of an Ag-rich layer on the outermost surface of the contact, which is considered to make the contact reliability of the contact unstable, an alloy made of Sn at a rate of 1 to 5% by weight, In at 3 to 10% by weight, one or two types of Fe, Ni and Co at 0.05 to 1% by weight and Ag for the remaining part is internally oxidized in Ag, and the Sn-In composite oxide of the added elements and oxides of one or two types of Fe, Ni and Co are uniformly and finely precipitated and dispersed in the internal structure.

Moreover, the present invention is characterized in that an oxide of In having a low steam pressure than CdO within a temperature range of approximately 500 to 4000°C is dispersed in Sn and Bi oxides, thereby making the behavior of a synthetic steam pressure of these oxides in the form of a metal composite oxide more approximate to the behavior of the steam pressure of CdO so that their synergistic effect provides excellent contact properties. The present invention is also characterized in that as a measure for restraining generation of an Ag-rich layer on the outermost surface of the contact, which is considered to make the contact reliability of the contact unstable, an alloy made of Sn at a rate of 1 to 5% by weight, In at 3 to 10% by weight, Bi at 0.05 to 2% by weight, one or two types of Fe, Ni and Co at 0.05 to 1% by weight and Ag for the remaining part is internally oxidized, and the Sn-In composite oxide, In-Bi composite oxide, Sn-Bi composite oxide and Sn-In-Bi composite oxide of the added elements and oxides of one or two types of Fe, Ni and Co are uniformly and finely precipitated and dispersed in the internal structure.

Moreover, the present invention is characterized in that an oxide of In having a low steam pressure than CdO within a temperature range of approximately 500 to 4000°C is dispersed in Sn and Sb oxides, thereby making the behavior of a synthetic steam pressure of these oxides in the form of a metal composite oxide more approximate to the behavior of the steam pressure of CdO so that their synergistic effect provides excellent contact properties. The present invention is also characterized in that as a measure for restraining generation of an Ag-rich layer on the outermost surface of the contact, which is considered to make the contact reliability of the contact unstable, an alloy made of Sn at a rate of 1 to 5% by weight, In at 3 to 10% by weight, Sb at 0.05 to 5% by weight, one or two types of Fe, Ni and Co at 0.05 to 1% by weight and Ag for the remaining part is internally oxidized, and the Sn-In composite oxide, In-Sb composite oxide, Sn-Sb composite oxide and Sn-In-Sb composite oxide of the added elements and oxides of one or two types of Fe, Ni and Co are uniformly and finely precipitated and dispersed in the internal structure.

Furthermore, the present invention is characterized in that an oxide of In having a lower steam pressure than CdO within a temperature range of approximately 500 to 4000°C is dispersed in Sn, Bi and Sb oxides, thereby making the behavior of a synthetic steam pressure of these oxides in the form of a metal composite oxide more approximate to the behavior of the steam pressure of CdO so that their synergistic effect provides excellent contact properties. The present invention is also characterized in that as a measure for restraining generation of an Ag-rich layer on the outermost surface of the contact, which is considered to make the contact reliability of the contact unstable, an alloy made of Sn at a rate of 1 to 5% by weight, In at 3 to 10% by weight, Bi at 0.05 to 2% by weight, Sb at 0.05 to 5% by weight, one or two types of Fe, Ni and Co at 0.05 to 1% by weight and Ag for the remaining part is internally oxidized, and the Sn-In composite oxide, In-Bi composite oxide, Sn-Bi composite oxide, Sn-Sb composite oxide, In-Sb composite oxide and Sn-In-Bi-Sb composite oxide of the added elements and oxides of one or two types of Fe, Ni and Co are uniformly and finely precipitated and dispersed in the internal structure.

As described above, an alloy made by solving Sn, In and one or two types of Fe, Ni and Co, and if necessary, one type or more of Bi and Sb, into Ag, is prepared in a desired contact shape at a processing rate of 50 to 95%, and after replacement with pure oxygen under a normal pressure, the temperature is raised from 200°C in an oxygen atmosphere with an oxygen pressure of 5 to 50 kg/cm² to set an internal oxidation temperature with an upper limit of 700°C. Thus, generation of an Ag-rich layer and an oxide-flocculated layer immediately below the Ag-rich layer, which are generated in the progress of internal oxidation of the conventional process, is restrained, and the internal dislocation density is increased by intense processing at the above-described high processing rate. By an interaction due to generation of many crystals and nucleuses for generating oxide particles, the composite oxides of the added elements are uniformly and finely precipitated and dispersed into the deep internal structure. This can provide a Cd-free electric contact having excellent electric properties such as deposition resistance, arc resistance and low contact resistance.

In the above description, the reason for setting the upper limit of the processing rate at 95% is that further processing is difficult in consideration of the limit of the processability of the material while processing at less than 50% is insufficient for generation of a sufficiently effective processing strain.

Moreover, the reason for the replacement with pure oxygen under a normal temperature and setting the oxygen pressure at 5 to 50 kg/cm² is that the replacement removes non-oxidative gases in the internal oxidation furnace, that is, nitrogen and hydrogen in the air, to improve the oxidation atmosphere in the furnace and that an oxygen pressure less than 5 kg/cm² is insufficient to realize uniform and fine precipitation and dispersion of the composite oxides of the added elements to the deep part in the material while an oxygen pressure equal to or higher than 50 kg/cm² increases the scale of the furnace facility and cannot provide an outstanding effect on the properties that matches the manufacturing cost.

Furthermore, the reason for raising the temperature from 200° in the pressured oxygen atmosphere and setting the internal oxidation temperature with the upper limit of 700°C is that 200°C is the lower limit of the temperature range of internal oxidation while at a temperature equal to or higher than 700°C, the diffusion rate of the solute element becomes higher than the diffusion rate of oxygen from the material surface in internal oxidation, thus forming solid layered flocculation on the surface layer of the structure and obstructing the subsequent progress of internal oxidation.

If the supply of pressured oxygen before the temperature rise is delayed, diffusion of the solute element starts in the state where diffusion of oxygen is insufficient, as in the above description, and the delay of supply of oxygen is considered to cause an oxide generation reaction on the surface layer of the structure and therefore deposition of an Ag-rich layer on the outermost surface.

Moreover, the reason for setting the upper limit of the content range of Sn with respect to Ag at 5% by weight is that addition exceeding this limit cannot realize fine precipitation of the oxide and forms solid layered flocculation inside the oxidized structure, thus obstructing the subsequent progress of internal oxidation and causing serious fragility in the oxidized structure. On the other hand, addition less than 1% by weight cannot satisfy composite oxidation with many elements and cannot provide an addition effect for sufficient electric properties.

Next, the reason for setting the upper limit of the content range of In at 10% by weight is that addition exceeding this limit forms a fine oxide coating on the surface in combination with the other elements at the time of internal oxidation and makes entry of oxygen from the surface difficult. Addition less than 3% by weight cannot realize the restraining effect on volatile damage and exhaustion due to an arc, that is, the effect of the above-described lower steam pressure than that of CdO.

Moreover, the reason for setting the upper limit of the content range of Bi at 2% by weight is that addition exceeding this limit causes hot fragility and makes it difficult to prepare an alloy for making a finer oxide, which is an element of the present invention, at a processing rate of 50 to 95%. In addition, such addition causes significant flocculation of the oxide at the time of internal oxidation and obstructs the subsequent progress of internal oxidation. Addition less than 0.05% by weight does not realize the effect to finely disperse the composite oxide particles.

The reason for setting the upper limit of the content range of Sb at 5% by weight is that addition exceeding this limit forms a fine oxide coating on the surface in combination with the other elements at the time of internal oxidation and makes entry of oxygen from the surface difficult. Addition less than 0.05% by weight does not realize the contact surface cleaning effect, which is the effect of the higher steam pressure than that of CdO.

Furthermore, the addition of one or two types of Fe, Ni and Co is effective mainly for making finer crystal grains and equalizing the oxide particle size. The reason for setting the upper limit of this addition at 1% by weight is that alloying by a melting method is extremely difficult even when addition exceeding this limit is performed, whereas addition less than 0.05% by weight cannot realize the effect to make finer crystal grains and the like.

### Brief Description of the Drawings

Fig.1 is a micrograph showing an internal structure of example 4 of the embodiment. Fig.2 is a micrograph showing an internal structure of conventional example 1.

### Best Mode for Carrying Out the Invention

To describe the present invention more in detail, examples of embodiment will be described with reference to the attached drawings and the following table 1 which is a chart showing electric properties with respect to structure alloys in the conventional example and examples of the embodiment.

Using Sn, In, Bi and Sb having purity of 99.5% by weight or higher and one or two types of Fe, Ni and Co as raw materials, composition alloys shown in Table 1 were prepared by the following process.

After an ingot melted and cast in a high-frequency induction melting furnace was hot-rolled, an Ag plate was bonded to one surface thereof by hot compression bonding to form an Ag layer for brazing.

Next, the material of each of examples 1 to 9 as shown in Fig. 3 was cold-rolled at each processing rate to form a plate with a thickness of 2 mm, and then a disc with a diameter of 6 mm was punched out.

In example 1, the temperature of this sample was raised to 200 to 600°C in an oxidation atmosphere with an oxygen pressure of 50 kg/cm², thus internally oxidizing the sample.

In example 2, the temperature was raised to 200 to 630°C in an oxidation atmosphere with an oxygen pressure of 30 kg/cm², thus internally oxidizing the sample.

In example 3, the temperature was raised to 200 to 550°C in an oxidation atmosphere with an oxygen pressure of 5 kg/cm², thus internally oxidizing the sample.

In example 4, the temperature was raised to 200 to 700°C in an oxidation atmosphere with an oxygen pressure of 50 kg/cm², thus internally oxidizing the sample.

In example 5, the temperature was raised to 200 to 670°C in an oxidation atmosphere with an oxygen pressure of 5 kg/cm², thus internally oxidizing the sample.

In example 6, the temperature was raised to 200 to 650°C in an oxidation atmosphere with an oxygen pressure of 20 kg/cm², thus internally oxidizing the sample.

In example 7, the temperature was raised to 200 to 600°C in an oxidation atmosphere with an oxygen pressure of 10 kg/cm², thus internally oxidizing the sample.

In example 8, the temperature was raised to 200 to 680°C in an oxidation atmosphere with an oxygen pressure of 8 kg/cm², thus internally oxidizing the sample.

In example 9, the temperature was raised to 200 to 450°C in an oxidation atmosphere with an oxygen pressure of 40 kg/cm², thus internally oxidizing the sample.

For comparison, an alloy containing Ag and 12% by weight of Cd as conventional example 1, an alloy containing Ag, 6% by weight of Sn and 3% by weight of In as conventional example 2, and an alloy containing Ag and 7% by weight of In as conventional example 3 were prepared and formed in a similar shape at a processing rate of 50% or less, and then internally oxidized at a fixed temperature of 780°C in an oxidation atmosphere with an oxygen pressure of 3 kg/cm². As a contact test, an actual machine test (AC 200V and 20A) was carried out using a contact resistor, a deposition tester (rated at 60A) and a commercially available contactor, and the electric properties were evaluated.

### Industrial Applicability

According to the present invention described above in detail, excellent electric properties such as deposition resistance, arc resistance and low contact resistance are provided, and ideal effects are shown in view of oxide particles and crystal grain diameter, as seen in the oxide structure of example 4 shown in Fig.1 and the oxide structure of conventional example 1 shown in Fig.2.

Moreover, the present invention is effective for removing the Ag-rich layer appearing on the outermost surface.

## Claims

1. A method for manufacturing an internal-oxidation-type Ag-oxide-based electric contact material, **characterized in that** after an atmosphere in a pressured oxidation furnace is replaced with oxygen, the temperature of an internal-oxidative Ag alloy prepared under a condition of a cold roll rate of 50 to 95% is gradually raised from a temperature of 200°C or less in a pressured oxygen atmosphere with an oxygen pressure of 5 to 50 kg/cm² and internal oxidation processing is performed with an upper limit temperature of 700°C , thereby restraining an Ag-rich layer generated on an outermost surface and an oxide-flocculated layer immediately below the Ag-rich layer and uniformly and finely precipitating and dispersing a composite oxide of added elements to a deep part of the internal structure.

2. The method for manufacturing an Ag-oxide-based electric contact material as claimed in claim 1, **characterized in that** the internal-oxidative Ag alloy prepared under the condition of a cold roll rate of 50 to 95% is an Ag alloy made of Sn, In, one or more types of Fe, Ni and Co, and Ag.

3. The method for manufacturing an Ag-oxide-based electric contact material as claimed in claim 1, **characterized in that** the internal-oxidative Ag alloy prepared under the condition of a cold roll rate of 50 to 95% is an Ag alloy made of Sn, In, one or more types of Bi and Sb, one or more types of Fe, Ni and Co, and Ag.

4. An Ag-oxide-based electric contact material made of Sn at a rate of 1 to 5% by weight, In at 3 to 10% by weight, Bi at 0.05 to 2% by weight, one or more types of Fe, Ni and Co at 0.05 to 1% by weight, and Ag for the remaining part, by the manufacturing method of claims 1 and 3.

5. An Ag-oxide-based electric contact material made of Sn at a rate of 1 to 5% by weight, In at 3 to 10% by weight, Sb at 0.05 to 5% by weight, one or more types of Fe, Ni and Co at 0.05 to 1% by weight, and Ag for the remaining part, by the manufacturing method of claims 1 and 3.

6. An Ag-oxide-based electric contact material made of Sn at a rate of 1 to 5% by weight, In at 3 to 10% by weight, Bi at 0.05 to 2% by weight, Sb at 0.05 to 5% by weight, one or more types of Fe, Ni and Co at 0.05 to 1% by weight, and Ag for the remaining part, by the manufacturing method of claims 1 and 3.

## Patentansprüche

1. Verfahren zur Herstellung aus auf Ag-Oxid basierenden elektrischen Kontaktmaterials mit innerer Oxidation,
**dadurch gekennzeichnet, dass** nach Ersatz einer Atmosphäre in einem unter Druck stehenden Oxidationsofen durch Sauerstoff die Temperatur einer Ag-Legierung mit innerer Oxidation, die unter einer Bedingung einer Kaltwalzrate von 50 bis 95 % hergestellt wurde, von 200°C oder weniger in einer unter Druck stehenden Sauerstoffatmosphäre mit einem Sauerstoffdruck von 5 bis 50 kg/cm² und einer inneren Oxidationsbehandlung auf eine obere Grenztemperatur von 700°C erhöht wird, wodurch die Bildung einer Ag-reichen Schicht auf einer äußersten Oberfläche und die Bildung einer ausgeflockten Oxidschicht unmittelbar unter der Ag-reichen Schicht verhindert werden und wodurch ein Verbundoxid von zusätzlichen Elementen an einem tiefen Teil der inneren Struktur gleichmäßig und fein ausgefällt und dispergiert wird.

2. Verfahren zur Herstellung eines elektrischen Kontaktmaterials auf Ag-Oxid-Basis nach Anspruch 1,
**dadurch gekennzeichnet, dass** die Ag-Legierung mit innerer Oxidation, die unter der Bedingung einer Kaltwalzrate von 50 bis 95% ausgewalzt wurde, eine Ag-Legierung ist, die aus Sn, In und einem oder mehreren Elementen von Fe, Ni und Co sowie Ag besteht.

3. Verfahren zur Herstellung eines elektrischen Kontaktmaterials auf Ag-Oxid-Basis nach Anspruch 1,
**dadurch gekennzeichnet, dass** die Ag-Legierung mit innerer Oxidation, die unter der Bedingung einer Kaltwalzrate von 50 bis 95% hergestellt wurde, eine Ag-Legierung ist, die aus Sn, In, einem oder mehreren der Elemente Bi und Sb und einem oder mehreren Elementen von Fe, Ni und Co sowie aus Ag besteht.

4. Elektrisches Kontaktmaterial auf Ag-Oxid-Basis, welches durch das Herstellungsverfahren gemäß den Ansprüchen 1 und 3 aus einer Legierung hergestellt wurde, die aus 1 bis 5 Gewichtsprozent Sn, 3 bis 10 Gewichtsprozent in, 0,05 bis 2 Gewichtsprozent Bi, 0,05 bis 1 Gewichtsprozent von einem oder mehreren der Elemente Fe, Ni und Co und als Rest aus Silber besteht.

5. Elektrisches Kontaktmaterial auf Ag-Oxid-Basis, welches durch das Herstellungsverfahren gemäß den Ansprüchen 1 und 3 aus einer Legierung hergestellt wurde, die aus 1 bis 5 Gewichtsprozent Sn, 3 bis 10 Gewichtsprozent In, 0,05 bis 5 Gewichtsprozent Sb, 0,05 bis 1 Gewichtsprozent von einem oder mehreren der Elemente Fe, Ni und Co und als Rest aus Silber besteht.

6. Elektrisches Kontaktmaterial auf Ag-Oxid-Basis, welches durch das Herstellungsverfahren gemäß den Ansprüchen 1 und 3 aus einer Legierung hergestellt wurde, die aus 1 bis 5 Gewichtsprozent Sn, 3 bis 10 Gewichtsprozent In, 0,05 bis 2 Gewichtsprozent Bi, 0,05 bis 5 Gewichtsprozent Sb, 0,05 bis 1 Gewichtsprozent von einem oder mehreren der Elemente Fe, Ni und Co und als Rest aus Silber besteht.

## Revendications

1. Procédé de fabrication d'un matériau de contact électrique à base d'Ag-oxyde à oxydation interne, **caractérisé en ce que**, après avoir remplacé une atmosphère, dans un four à oxydation pressurisé, par de l'oxygène, la température d'un alliage d'Ag à oxydation interne, préparé à une vitesse de laminage à froid de 50 à 95 %, est graduellement augmentée à partir d'une température de 200°C ou inférieure dans une atmosphère d'oxygène sous pression avec une pression d'oxygène de 5 à 50 kg/cm² et un processus d'oxydation interne est mis en oeuvre avec une limite supérieure de température de 700°C, de cette façon limitant une couche riche en Ag générée sur une surface la plus à l'extérieur et une couche floculée d'oxyde immédiatement au-dessous de la couche riche en Ag et précipitant et dispersant de manière uniforme et fine un oxyde composite des éléments ajoutés dans une partie profonde de la structure interne.

2. Procédé de fabrication d'un matériau de contact électrique à base d'Ag-oxyde selon la revendication 1, **caractérisé en ce que** l'alliage d'Ag à oxydation interne, préparé à une vitesse de laminage à froid de 50 à 95 %, est un alliage d'Ag constitué de Sn, d'In, d'un ou plusieurs types de Fe, Ni et Co, et d'Ag.

3. Procédé de fabrication d'un matériau de contact électrique à base d'Ag-oxyde selon la revendication 1, **caractérisé en ce que** l'alliage d'Ag à oxydation interne, préparé à une vitesse de laminage à froid de 50 à 95 %, est un alliage d'Ag constitué de Sn, d'In, d'un ou plusieurs types de Bi et de Sb, d'un ou plusieurs types de Fe, Ni et Co, et d'Ag.

4. Matériau de contact électrique à base d'Ag-oxyde constitué de Sn à un taux de 1 à 5 % en poids, d'In à un taux de 3 à 10 % en poids, de Bi à un taux de 0,05 à 2 % en poids, d'un ou plusieurs types de Fe, Ni et Co à un taux de 0,05 à 1 % en poids, et d'Ag pour la partie restante, par le procédé de fabrication selon les revendications 1 et 3.

5. Matériau de contact électrique à base d'Ag-oxyde constitué de Sn à un taux de 1 à 5 % en poids, d'In à un taux de 3 à 10 % en poids, de Sb à un taux de 0,05 à 5 % en poids, d'un ou plusieurs types de Fe, Ni et Co à un taux de 0,05 à 1 % en poids, et d'Ag pour la partie restante, par le procédé de fabrication selon les revendications 1 et 3.

6. Matériau de contact électrique à base d'Ag-oxyde constitué de Sn à un taux de 1 à 5 % en poids, d'In à un taux de 3 à 10 % en poids, de Bi à un taux de 0,05 à 2 % en poids, de Sb à un taux de 0,05 à 5 % en poids, d'un ou plusieurs types de Fe, Ni et Co à un taux de 0,05 à 1 % en poids, et d'Ag pour la partie restante, par le procédé de fabrication selon les revendications 1 et 3.
